

June 25, 1957

H. B. LAW ET AL

2,797,331

ELECTRON-SENSITIVE PHOTOGRAPHIC PLATE

Filed March 18, 1952

*Fig. 1.*



*Fig. 2.*



INVENTORS  
HAROLD B. LAW  
JOHN E. EVANS  
& NATHAN RYNN  
BY

W.S. Hill  
AGENT

## 1

2,797,331

## ELECTRON-SENSITIVE PHOTOGRAPHIC PLATE

Harold B. Law, Princeton, John E. Evans, Montgomery Township, Somerset County, and Nathan Rynn, Princeton, N. J., assignors to Radio Corporation of America, a corporation of Delaware

Application March 18, 1952, Serial No. 277,132

18 Claims. (Cl. 250—49.5)

This invention relates, in general, to electron-sensitive photographic plates and, more particularly, to plates which are capable of recording electron images but which are relatively insensitive to ordinary visible light.

It has been found desirable to have some method of photographing images produced by electron optical systems where the electrons are generated by a thermionic emitter. This problem arises, for example, in plotting the positions at which phosphor dots are to be deposited on the viewing screen of one type of tri-color television kinescope tube. One method utilized for plotting the positions of the dots is to expose a photographic plate, through an electron-focusing grid of crossed wires, to a thermionically generated beam of electrons scanned across the area of the plate. The grid of wires has apertures to permit passage of the electron beam wherever it is desired to place a phosphor dot on the completed screen. After the photographic plate has been properly exposed to the electron beam to form a multiplicity of latent dot images, the plate is developed and a print is then made on a medium which is to be used for actual printing of the phosphor dots on a base member. This method of plotting is more fully described and claimed in a copending application of Harold B. Law, Serial No. 277,133, filed concurrently herewith and now Patent 2,727,828.

In developing the above described process, it was found that ordinary types of photographic plates are not suitable for at least two reasons. One reason is that a thermionic emitter generates visible light. An ordinary photographic plate is exposed immediately by the light and rendered useless to record electron optical images. Another reason is that an ordinary photographic plate is a good electrical insulator and, when exposed to an electron beam, accumulates an electrical charge which has an undesirable effect on the characteristics of the electron optical lens system which is used to plot the position of the phosphor dots. It was, therefore, found necessary to devise a photographic plate which was, initially, at least, sensitive to record electron optical images but relatively insensitive to visible light and was, at the same time, a fairly good electrical conductor.

One object of the present invention is to provide a photographic plate which is sensitive to electrons, electrically conductive, and relatively insensitive to ordinary visible light of predetermined wavelengths.

Another object of the invention is to provide a photographic plate which is sensitive to electrons but relatively insensitive to the light generated by a thermionic emitter.

Another object of the invention is to provide an improved photographic plate for recording images formed in electron optical systems.

Still another object of the invention is to provide an improved electron sensitive photographic plate which can be used in an electron optical system without having any undesirable effects on the lens characteristics of the system.

These and other objects will be more apparent and the

## 2

invention will be more readily understood from the following detail description and the illustrative drawing of which:

Fig. 1 is a perspective view of one embodiment of a photographic plate constructed in accordance with the principles of the present invention; and

Fig. 2 is a cross-section view taken through the line II—II of Fig. 1.

In general, the present invention comprises an improved photographic plate and methods of making the improved plate. The plate comprises a base member having disposed on a surface thereof a layer of conventional photographic material which is also electron sensitive. The photographic material is covered with an electrically conducting coating and is also provided with a light filtering substance capable of filtering out most of the light in the visible wavelengths to which the photographic material is sensitive. For particular purposes, the exposed surface of the photographic material may be provided with an electrode.

A preferred example of method of preparation of a preferred embodiment of a photographic plate in accordance with the principles of the present invention will now be given.

The improved type of photographic plate of the present invention may be made by modifying a conventional plate comprising a transparent glass base member having one surface coated with a gelatin emulsion containing silver halide salts, for example, silver bromide and silver iodide. Plates of the kind which are suitable are sold under the trade name "Kodalith." In the first step of the modification process, the surface of the gelatin emulsion is treated, in the dark, by wetting it with an aqueous suspension of graphite (Aquadag). This suspension may be prepared by mixing the graphite and water in the proportion of about 1 gm. of the former per 100 cc. of the latter. This proportion is not at all critical, however, and any other convenient proportions may be selected from which a thin, even coating of the graphite can be deposited. In the wetting process, the suspension is briskly agitated to obtain an even distribution. Excess suspension is poured off the surface of the plate and the plate is permitted to drain. This provides a very thin, light-transmitting coating of graphite on the surface of the emulsion. This coating has a very high electrical resistance.

The second step of the process is to impregnate the gelatin emulsion with a red organic dye. This may be done by making up a saturated aqueous solution of Basic 50 Fuchsin dye (.335 gm./liter) and soaking the graphite coated plate in the solution for about 5 minutes. The surface of the plate is then rinsed and dried.

Next, the graphite-coated surface of the plate is rendered more conductive by gently polishing or burnishing with a piece of soft material, such as absorbent cotton. The burnishing action apparently causes the graphite particles to overlap and touch each other at a sufficient number of points to lower the electrical resistance of the surface to a considerable extent.

The plate which is made as described above is complete so far as some applications are concerned. However, if the plate is to be used to record dot-images in the process of manufacturing certain types of tri-color television kinescope tube viewing screens, it is necessary to maintain it at a particular potential. In order to do this, an electrode should be applied to the coated surface of the plate. This may be done by painting an air-drying silver paste in the form of a stripe around the edges of the coated surface. The paste may comprise, for example, a colloidal suspension of silver in an organic medium including a volatile organic solvent. The organic

medium may be, for example, nitrocellulose in amy1 acetate.

A plate, as made by the above described example of the process of the present invention, is shown in the drawings. In the figures, a glass plate 2 carries on one of its surfaces a layer 4 of gelatin emulsion containing silver halide salts. The emulsion is impregnated with a red dye and has its outer surface 8, which is the one opposite the glass plate 2, covered with an electrically conducting coating of graphite 10. This coating is just thick enough to be a fairly good electrical conductor but is not thick enough to prevent passage of light. When held up to the light (after the plate is developed), the appearance of the graphite coating is that of lightly smoked glass. Its surface resistivity should preferably be from 1 to 10 megohms. The completed plate which is illustrated also includes a silver paste electrode 12 in the form of a stripe around the edges of the coated surface 8.

A method of utilizing the photographic plate which has been described above is described and claimed in the previously mentioned copending application of Harold B. Law. As explained in the copending application, the plate may be exposed to an electron beam which is generated by a thermionic emitter such as a glowing wire filament. The filament gives off visible light within a broad range of wavelengths in the visible portion of the spectrum. Ordinary photographic emulsion, such as that described herein, are relatively insensitive to light in the red region of the visible spectrum but are sensitive to light in the other regions. In the present case, however, the red dye filters out nearly all of the light in the visible wavelengths, except the red rays, and thus renders the photographic emulsion relatively insensitive to all visible wavelengths to which it would otherwise be sensitive. In the case of the preferred example described, sensitivity of the plate was reduced to about one-hundredth its normal value.

Exposure of the photographic plate to a focused electron beam from the thermionic emitter produces a latent image wherever the beam strikes the emulsion. The plate is later developed in conventional manner to bring out a visible image. This may be printed on any conventional photographic printing medium by exposing to an ordinary incandescent lamp. The exposure is somewhat longer than usual since much of the red dye is still present in the plate after developing and washing.

Complete insensitivity to light of most visible wavelengths is not desired in this case since printing registration marks are put on the plate by exposure to light rather than electrons. Electrons could also be used for this but light is more convenient.

Many variations may be made in the photographic plate of the present invention without departing from the scope of the invention. The base member may be some transparent medium other than glass, for example, mica or synthetic resins. Also, the base member need not be transparent if printing of the image is done by reflected light. In this case, the member may be a metal, such as aluminum, or metal coated with enamel.

The photosensitive emulsion may be any one of hundreds of conventional compositions. Although gelatin containing silver halide salts is preferred to obtain good contrast, the material may comprise merely bichromated gelatin, or gelatin with cerium salts. Also, the suspending medium may be collodion (nitrocellulose) or other film forming materials in which light-sensitive materials can be incorporated. The particular photosensitive material used is not critical.

The particular substance used to render the photographic plate insensitive to ordinary visible light depends partially on the composition of the photosensitive material utilized. Since most photosensitive materials are usually sensitive to all wavelengths in the visible portion of the spectrum except red, the light filtering substance should usually be

a red organic dye. Many different red organic dyes may be used, for example, Eosin, Neutral Red, Saffronine, Rose Bengal, and Alizarin Red S. Any red organic dye can be used which does not have an unfavorable reaction with the photosensitive coating material. If it is desired to use a light sensitive material which is insensitive to wavelengths other than red, some other colored dye can be used.

The light filtering material need not be impregnated in the photographic emulsion. It may be applied as a surface coating only, for example. This is more desirable if the photographic material is a suspension in collodion rather than gelatin.

The electrically conductive coating also does not have to be graphite. It may, for example, be a thin, light transmitting coating of a metal such as aluminum applied by evaporation in vacuo. If applied in this manner, the heating filament must, of course, be shielded from the photographic plate in such a manner that no light from the filament reaches the plate.

What is claimed is:

1. A photographic plate comprising a base member having on a surface thereof a layer of electron-sensitive photographic material, said layer having on at least the surface opposite said member a stratum of light filtering material comprising an organic dye capable of preventing the passage of substantially all light of predetermined wavelengths in the visible portion of the spectrum, said filtering material being substantially transparent to the passage of electrons, and also having a stratum of light-transmitting electrically conducting material.

2. A plate according to claim 1 in which said base member is light transmitting.

3. A plate according to claim 1 in which said photographic material is a gelatin emulsion containing a photo-sensitive material.

4. A plate according to claim 3 in which said gelatin emulsion contains a silver halide salt.

5. A plate according to claim 1 in which said dye is a red dye.

6. A plate according to claim 5 in which said dye is Basic Fuchsin.

7. A plate according to claim 1 in which said electrically conducting material is carbon.

8. A photographic plate comprising a glass plate having on a surface thereof a layer of photographic emulsion, said emulsion having sufficient red organic dye impregnated therein to exclude substantially all visible light in the blue and green portions of the spectrum and having on the surface thereof an electrically conducting, light-transmitting coating of graphite.

9. A plate according to claim 8 in which said red dye is Basic Fuchsin.

10. A method of making a photographic plate comprising applying to a surface of a plate a layer of electron-sensitive photographic material, applying to the surface of said photographic material a stratum of electrically conducting, light-transmitting material, and impregnating at least part of said layer of photographic material with an organic dye capable of filtering out substantially all visible light of all of the wavelengths to which said photographic material is sensitive.

11. A method according to claim 10 in which said electron-sensitive photographic material is a gelatin emulsion containing a silver halide salt.

12. A method according to claim 11 in which said electrically conducting material is graphite.

13. A method according to claim 12 in which said graphite is applied to the surface of said emulsion in the form of a water suspension, the plate is then dried and the surface is burnished in order to decrease the electrical resistance thereof.

14. A method according to claim 13 in which said dye is applied to the graphite coated surface of said

plate in the form of a water solution, before said polishing step.

15. A method according to claim 14 in which said dye is a red dye.

16. A method of rendering a photographic plate suitable for recording images in an electron optical system where the electron source is a thermionic emitter, comprising applying an electrically conducting, light-transmitting coating to the sensitive surface of said plate and treating the photosensitive material of said plate with a light filtering organic dye capable of filtering out substantially all visible light of all wavelengths to which said photosensitive material is sensitive.

17. A photographic plate comprising a base member having on a surface thereof a layer of electron-sensitive photographic material, said layer having on at least the surface opposite said member a stratum of light filtering material comprising an organic dye capable of prevent-

ing the passage of substantially all visible light of predetermined wavelengths, said plate also including at least a surface stratum of electrically conducting, light-transmitting material, and an electrode making good electrical contact with a portion of said electrically conducting material.

18. A plate according to claim 17 in which said electrode is a coating of metallic paste adjacent the edges of said electrically conducting material.

10

References Cited in the file of this patent

UNITED STATES PATENTS

|           |                      |                |
|-----------|----------------------|----------------|
| 816,172   | Morse et al. -----   | Mar. 27, 1906  |
| 1,973,886 | Scanlan et al. ----- | Sept. 18, 1934 |
| 2,372,170 | Baker -----          | Mar. 27, 1945  |
| 2,446,248 | Schrader -----       | Aug. 3, 1948   |
| 2,542,304 | Boucher -----        | Feb. 20, 1951  |